

May 7, 1935.

A. C. WALKER

2,000,428

ELECTRICAL CONDUCTOR

Filed Jan. 9, 1932

FIG. 1



FIG. 2



FIG. 3



## UNITED STATES PATENT OFFICE

2,000,428

## ELECTRICAL CONDUCTOR

Albert C. Walker, East Orange, N. J., assignor to  
 Bell Telephone Laboratories, Incorporated,  
 New York, N. Y., a corporation of New York

Application January 9, 1932, Serial No. 585,759

7 Claims. (Cl. 173—264)

This invention relates to insulated conductors and particularly to flexible insulated conductors and cables and the method of their manufacture. The invention is especially applicable to insulated 5 conductors such as are used in telephone switch-board cables and to distributing frame wire, both of which are used extensively in the telephone plant.

It is well-known that different insulating materials vary widely in their electrical properties, such as insulation, resistance and capacity. Fibrous materials such as cotton and tussah floss silk which are used extensively in the insulation of flexible conductors possess good electrical 10 properties when dry but when these materials are exposed to moist air their insulation resistance is considerably lowered and their capacity increased. Regardless of their relative insulating properties the insulation resistance of all such 15 materials falls off rapidly under rising humidity conditions. While the amount of water absorption is not necessarily a direct and proportionate measure of the insulation resistance of fibrous insulating materials, nevertheless the presence of 20 water in all cases produces a deleterious effect upon the insulation resistance properties. The presence of absorbed water in switchboard cable insulation causes unbalances and short-circuit paths between the various conductors, thus destroying their efficiency for purposes of telephonic 25 communication, and also sets up an electrolytic action which tends to decompose the conductors and may ultimately render the cable unfit for service.

The principal object of the present invention 30 is to improve the electrical characteristics of insulated conductors and to maintain these improved characteristics even when the conductors are exposed to moist air.

Another object of the invention is to maintain 35 the improved electrical characteristics with a structure which is relatively flexible and one that has an improved appearance and can be manufactured economically.

To attain these objects and in accordance with 40 a feature of the invention, the conducting core is provided with a plurality of coatings of cellulose acetate of different derivatives. The inner coating may comprise one or more layers of 45 fibrous material such as cotton which has been converted into the lower derivatives of cellulose acetate and in which the individual fibres are similar in many of their physical characteristics to the fibres of the original material. By thus 50 acetylating the fibrous material, its electrical properties are greatly enhanced and its attraction for atmospheric moisture is diminished. After being provided with a coating of cellulose acetate of the lower derivatives, the insulated 55 wire is preferably first treated to expel any mois-

ture present and is then treated with a cellulose acetate lacquer comprising a suitable solvent such as acetone and a homogeneous cellulose acetate of a higher derivative such as cellulose triacetate, after which it is passed through a 5 drying chamber which dries off all traces of the solvent. Since the lacquer and the acetylated fibrous material are both forms of cellulose acetate, they possess a high affinity for each other and are bonded together in such a way as to form 10 a coating about the conductor which is flexible, has a good appearance and is water repellent to a high degree. As the coating of cellulose acetate lacquer dries, there is a shrinking down of 15 the fibres and as a result the diameter of the completely insulated conductor is less than that of the conductor before the final treatment and individual loose fibre ends are matted down and therefore do not present leakage paths. Accordingly 20 the insulation resistance of a conductor made in this manner is far superior to that of any flexible conductor made heretofore where fibrous materials are employed and the capacity is decreased accordingly.

The invention may be more clearly understood 25 by reference to the accompanying drawing in which:

Fig. 1 discloses an electrical cable embodying the features of this invention;

Fig. 2 is a view illustrating the method employed in impregnating the individual conductors; and

Fig. 3 illustrates two portions of an insulated conductor one of which is untreated and the other of which is treated in accordance with this 35 invention.

Referring to Fig. 1, there is disclosed an electrical cable in which a plurality of bare conductors 5, 5 each of which is insulated with servings 6 and 7 of acetylated cotton wound on with reverse twists and the conductors as thus formed are then impregnated with cellulose acetate. The conductors thus insulated are twisted in pairs and grouped together by means of a spaced serving of cotton yarn 8 and a spirally wrapped 40 paper strip 9 over which is wrapped a metal tape 10, and braided fabric covering 11.

The cotton or other fibrous cellulose material which is to be placed about the bare conductor is first converted into cellulose acetate of the 45 lower derivatives in which form the individual fibres retain their physical characteristics but their electrical characteristics are greatly improved. Preferably the cotton or other fibrous material is first soda-boiled and subjected to a 50 bleaching process which reduces the ash content of the material and removes the natural waxes present, thereby permitting more uniform acetylation. Particularly good results have been ob- 55

tained when the following process has been employed prior to acetylation:

(1) Heat 2½ parts of cotton with 40 parts by weight of 1½% to 2% caustic soda solution for 5 to 4 hours at approximately 300° F. in the absence of air.

(2) Wash free from alkali with water.

(3) Bleach for 2 hours with 50 parts of a .1% calcium hypochlorite solution (35% available chlorine) by weight at room temperature (60 to 85° F.).

(4) Wash well.

(5) Treat for 1 hour with 50 parts of water containing .02% part of concentrated sulphuric acid, to destroy traces of the hypochlorite.

(6) Wash.

(7) Allow to stand 1 hour at room temperature in 40 parts water containing .01 part sodium bisulfite ( $\text{Na}_2\text{HSO}_3$ ) to effect dechlorination.

(8) Wash.

(9) Dry quickly at room temperature (120° F.).

The bleached material is next acetylated to yield a product varying in acetyl value from 10% to about 35% depending upon the variation in the time of acetylation and the temperature and combustion of the acetylating bath. In general, the most desirable results both electrically and mechanically are obtained when the acetylation process is not carried beyond the stage where the material is converted into mono-acetate the theoretical acetyl value of which is 21.1% but good results are obtained when the product consists of di-acetate, the acetyl value of which is 34.9%, or a combination of mono-acetate and di-acetate. If the acetylation is carried beyond the di-acetate stage destruction of the fibres occurs to such an extent that the mechanical strength of the product is decreased and it is much less satisfactory. Furthermore, the mono-acetate and di-acetate obtained by partial acetylation are insoluble in ordinary organic solvents such as acetone, chloroform, the benzene, the alcohols and also the acetylating mixture itself.

A typical example of the acetylating process and one which has been found to give particularly good results is as follows: The bleached cotton yarn is immersed in 8.8 times its weight of acetylating mixture which contains 4 parts commercial glacial acetic acid, 4 parts commercial acetic anhydride (90 to 95%) and .8 part commercial anhydrous zinc chloride, for 7 hours at 25° C. The excess acid is removed by wringing or centrifuging and the cotton is immersed in or flooded with a large volume of water, washed acid free, and dried. The material obtained by following this process has an acetyl value of about 17%. It is necessary to control the temperature within very narrow limits as, for example, 60/2 yarn acetylated under the same conditions as described above at various temperatures yields the following acetyl values:

| Temperature—<br>degrees C. | Acetyl values |
|----------------------------|---------------|
| 22                         | 12            |
| 24                         | 16            |
| 26                         | 18            |
| 28                         | 22            |
| 30                         | 26            |

While cotton has been cited as an example and it is believed that this material lends itself most readily for the insulation of electrical conductors, the process may also be employed on other cellulose materials such, for example, as flax, ramie,

hemp, etc., the essential feature being to insure that the acetylating process is not carried beyond the di-acetate stage and preferably not beyond the mono-acetate stage.

After the conductor has been provided with one or more servings of partially acetylated cellulose material it is coated or impregnated with a cellulose acetate of a higher derivative (cellulose tri-acetate). Both of these coverings being formed of cellulose acetate, they possess a high affinity for each other and as a result are bonded together so as to form an insulating coating about the conductor which is not only flexible but one which is water repellent to a high degree and, therefore, one which possesses superior electrical characteristics when exposed to moisture. In applying the outer coating of cellulose tri-acetate it is preferable to maintain the temperature of the coated wire above the dew point until the solvent has evaporated, thus leaving an outer glossy tube-like coating which possesses high insulation resistance under substantially all humidity conditions up to the dew point.

Referring to Fig. 2 of the drawing the supply reel 15, upon which is wound the conductor provided with a serving of cellulose acetate of the lower derivatives, is heated to expel all moisture prior to the impregnating process. From the supply reel the conductor passes through an inlet 16 provided with a stuffing box 1 into the impregnating tank 17 containing a bath of cellulose tri-acetate dissolved in acetone or other suitable solvent. As the conductor enters tank 17 it passes over guide roller 18 and is then directed through the impregnating bath by guide rollers 19, 20, 21. The coated conductor emerges from the tank through a small vent 22 in the air-tight cover 23 and into the drying chamber 24. If desired, the vent 22 may be equipped with a die or wiper for removing all excess solution from the impregnated conductor. A strong current of hot dry air is circulated through the chamber 24 from an inlet pipe 25 to an outlet pipe 26 which may be associated with condensing apparatus (not shown) for recovering the solvent. The hot dry air is preferably maintained at or above the temperature of the boiling point of acetone or other solvent employed and the temperature may be observed at all times by means of a thermometer 27 associated with the inlet pipe 25.

The acetone content in the insulation is rapidly evaporated in chamber 24 leaving a glossy coating upon the fibrous insulation. After passing over a suitable guide roller 28 and through an outlet 29 provided with a stuffing box, the conductor emerges from chamber 24 and is wound upon the take-up reel 30.

A die or wiper may be mounted at outlet 29 for the purpose of removing uneven particles of cellulose acetate which may tend to cling to the surface of the insulation, thus giving a smooth or polished appearance to the conductor. The evaporation of the acetone in chamber 24 leaves a moisture resisting, insulated cover upon the wire in which the fibres of cellulose acetate of the lower derivatives are enclosed in a matrix of cellulose tri-acetate and intimately bonded thereto. The cellulose tri-acetate in drying causes a shrinking down of the fibres and produces a solid tube-like insulation which is considerably smaller in diameter than the original unimpregnated loose insulation. This is illustrated more clearly in Fig. 3 in which 31 is a magnified section of unimpregnated insulation showing the presence of loose fibres projecting there-

from which form leakage paths when the conductors are grouped together in a cable. Upon being impregnated with cellulose tri-acetate these fibres are matted down as shown at 32, thus materially reducing the space occupied by the insulation and permitting a greater bulk of conductors to be enclosed in a given space in a cable sheath when capacity considerations admit of it. At the same time the area and points of contact between the insulated conductors are decreased, thus decreasing the leakage paths between conductors.

The results of a large number of tests made with conductors insulated with partially acetylated cotton indicate that the resulting insulation resistance under similar conditions is from 500 to 1000 times that of purified cotton and about 10 times that of purified silk. For use in toll cables it is required that the insulating material not only have a high insulation resistance but also that it have a low capacitance and conductance. The tests show that a toll conductor provided with two servings of partially acetylated cotton and a coating of cellulose tri-acetate has an insulation resistance of from 6 to 12 times that of a standard type of toll cable employing two servings of purified silk and a coating of cellulose tri-acetate. The capacitance of the cable employing acetylated cotton is only 80% that of the standard cable while the conductance is 30% of the standard cable and the capacitance unbalance is only 30% of that obtained from the standard cable. These results indicate that not only is it possible to replace the highest grade of silk insulation employed on toll cables with acetylated cotton but that a far superior product results.

For other types of cables the conductance and capacitance unbalance requirements are not so severe and, therefore, in certain cases it may be found desirable to replace the outer serving 7 with a serving of purified cotton. By this means it is possible to obtain a cable having electrical characteristics superior to those now available and at a somewhat lower cost since the purified cotton is somewhat cheaper than the acetylated cotton and it is more economical to dye.

What is claimed is:

1. An electrical conductor comprising a conducting core, an insulated coating of partially acetylated cellulose having an acetyl value not

greater than 35% surrounding said core and an outer coating of cellulose acetate having an acetyl value not less than 37% in intimate contact with and bonded to said inner coating.

2. An electrical conductor comprising a conducting core, a coating of fibrous cellulose acetate of the lower derivatives surrounding said core and a coating of non-fibrous cellulose acetate surrounding and bonded to said first coating.

3. An electrical conductor comprising a conducting core, a coating of partially acetylated cellulose fibres surrounding said core and an outer coating of completely acetylated cellulose in intimate contact with said inner coating and shrinking down the individual fibres thereof.

4. An electrical conductor comprising a conducting core, a coating about said core of partially acetylated cellulose non-soluble in the ordinary organic solvents, and an outer coating of cellulose acetate of a form soluble in said organic solvents surrounding and bonded to said inner coating.

5. An electrical conductor comprising a conducting core, a coating about said core of partially acetylated cotton fibres having an acetyl value of approximately 20% and an outer coating of cellulose tri-acetate enclosing said fibres in a matrix of cellulose tri-acetate and bonded thereto.

6. An electrical conductor comprising a conducting core, a coating of partially acetylated cotton helically wrapped about said core, a second coating of acetylated cotton helically wrapped about said first coating with a reverse twist, and a coating of cellulose tri-acetate bonded to and surrounding said second coating.

7. An electrical cable comprising a plurality of pairs of twisted conductors each of said conductors being insulated with an inner coating of partially acetylated cellulose and an outer coating of cellulose tri-acetate bonded to said first coating, and shrinking down the outer fibers of the partially acetylated cellulose to prevent leakage paths between adjacent conductors, and a spaced serving of fibrous cellulose binding said conductors in the form of a cable.

ALBERT C. WALKER. 50